

# United States Patent [19]

Yanagida et al.

[11] 3,929,612

[45] Dec. 30, 1975

[54] **PROCESS FOR ELECTROLYTICALLY COLORING THE ANODICALLY OXIDIZED COATING ON ALUMINUM OR ALUMINUM BASE ALLOYS**

|           |        |                    |          |
|-----------|--------|--------------------|----------|
| 3,634,208 | 1/1972 | Kuroda .....       | 204/35 N |
| 3,759,801 | 9/1973 | Patrie.....        | 204/35 N |
| 3,761,362 | 9/1973 | Oida .....         | 204/35 N |
| 3,788,956 | 1/1974 | Patrie et al. .... | 204/35 N |
| 3,798,137 | 3/1974 | Kampert .....      | 204/35 N |

[75] Inventors: **Kiyomi Yanagida; Tadashi Hirokane; Tadashi Tsukiyasu; Tomoari Sato**, all of Nagoya, Japan

*Primary Examiner*—John H. Mack  
*Assistant Examiner*—Aaron Weisstuch  
*Attorney, Agent, or Firm*—Sughrue, Rothwell, Mion, Zinn & Macpeak

[73] Assignee: **Sumitomo Chemical Company, Limited**, Osaka, Japan

[22] Filed: **Oct. 21, 1974**

[21] Appl. No.: **516,523**

[30] **Foreign Application Priority Data**

Oct. 20, 1973 Japan..... 48-118047

[52] **U.S. Cl..... 204/35 N**

[51] **Int. Cl.<sup>2</sup>..... C25D 5/48**

[58] **Field of Search..... 204/35 N, 58, 42**

[56] **References Cited**

UNITED STATES PATENTS

3,616,297 10/1971 Cooke et al. .... 204/35 N

[57]

## ABSTRACT

In the process for electrolytically coloring an anodically oxidized coating on an aluminum or aluminum base alloy article by subjecting the anodized aluminum or aluminum base alloy article as a cathode to an electrolytic coloring treatment with a direct current in an electrolytic coloring bath containing a nickel salt, an improvement which comprises conducting the electrolytic coloring treatment at a pH in the range of from 2.0 to 5.5 to obtain a uniformly colored film.

**8 Claims, No Drawings**

**PROCESS FOR ELECTROLYTICALLY COLORING  
THE ANODICALLY OXIDIZED COATING ON  
ALUMINUM OR ALUMINUM BASE ALLOYS**

**BACKGROUND OF THE INVENTION**

**1. Field of the Invention**

The present invention relates to a process for coloring an anodically oxidized coating on an aluminum or aluminum base alloy article (hereinafter referred to as "aluminum" for brevity). More particularly, the invention relates to a process for electrolytically coloring an aluminum article which has previously been anodically oxidized, which comprises subjecting the anodically oxidized aluminum as a cathode to an electrolytic coloring treatment with a direct current in an electrolytic coloring bath containing a nickel salt to obtain a uniformly colored film.

**2. Description of the Prior Art**

It was known that an electrolytic coloring bath containing a nickel salt can provide uniformly colored films in a stable manner at a low cost and, therefore, the electrolytic coloring bath is quite suitable for the operation on an industrial scale. Furthermore, when an electrolytic coloring bath containing a nickel salt is used, a wide variety of colors, i.e., from yellow brown, light brown to dark brown can be obtained and the colors obtained are excellent in uniformity and color reproducibility.

However, when an aluminum article is electrolytically colored in the electrolytic coloring bath containing a nickel salt on an industrial scale, a phenomenon sometimes occurs such that only a faint color is formed or the colored film tends to be peeled, i.e., so-called "oxide-spalling" may occur, and thus it is difficult to obtain a uniformly colored film on the aluminum articles in a stable manner.

**SUMMARY OF THE INVENTION**

As the result of various investigations, it has been found that the deviation in the pH value of the electrolytic coloring bath is one of the main causes of the above-described difficulties. That is, if the pH value of the electrolytic coloring bath becomes lower than 2.0, the color of the film on aluminum articles becomes quite faint and a sufficiently deep color which is practically useful cannot be obtained even if the electrolytic coloring treatment is effected for a prolonged period of time and, on the other hand, if the pH value of the electrolytic coloring bath becomes higher than 5.5, a film having only faint color is obtained and, in addition, the film formed tends to peel during the coloring treatment.

A primary object of this invention is to provide an improved process for electrolytically coloring an anodically oxidized coating on an aluminum by subjecting the aluminum having the anodized oxide film in a thickness of at least 6 microns thickness to a direct current electrolysis as a cathode in an electrolytic coloring bath containing a nickel salt, the improvement comprising conducting the electrolytic coloring treatment in an electrolytic coloring bath at a pH in the range of 2.0 to 5.5.

**DETAILED DESCRIPTION OF THE INVENTION**

The purpose of the first anodic oxidation treatment of this invention is the formation of a practically useful anodically oxidized coating on the surface of the alumi-

num and, in particular, the anodically oxidized coating having a thickness of at least 6 microns which has been formed on the aluminum in an anodic oxidation bath containing sulfuric acid and/or an aromatic sulfonic acid as a main component can be uniformly colored with the electrolytic coloring treatment in a stable manner and further the colored film has high weatherability. For the formation of the anodically oxidized coating on the aluminum, an aqueous sulfuric acid solution

having a concentration of from about 10 to 30% by weight, preferably 10 to 20% by weight is usually used as the anodic oxidation bath and an aluminum article is subjected to the anodizing treatment with a direct current at room temperature (about 20°-30°C) and a current density of about 1 ampere/dm<sup>2</sup> or, occasionally, at a higher current density of 3.0 to 5.0 amperes/dm<sup>2</sup>. However, stable coloring treatment can be attained when the above anodizing conditions, i.e., sulfuric acid concentration, current density and bath temperature are changed to some extent, so long as the thickness of the anodically oxidized coating formed on the aluminum article is above 6 microns. Also, when an anodic oxidation bath containing an aromatic sulfonic acid as the main component is used, the anodization is preferably conducted in an aqueous solution of the aromatic sulfonic acid having a concentration of about 10% by weight by superimposing an alternating current on a direct current.

The coloring treatment of the anodized article is then carried out without applying a sealing treatment by a direct current electrolysis using the aluminum article as a cathode in an aqueous solution containing a nickel salt as an electrolytic coloring bath.

The electrolytic coloring bath used in this invention contains a water-soluble nickel salt as the main component and the electric conductivity of the bath can usually be controlled by adding thereto an appropriate amount of boric acid, sulfuric acid, etc. Examples of the water-soluble nickel salt are nickel sulfate, nickel chloride and nickel acetate, and the concentration of the nickel ion as the main component of the electrolytic coloring bath can vary over a wide range. For example, when nickel sulfate is used as the nickel salt, a desired colored film is obtained at a nickel sulfate concentration of 15 to 100 g/liter. Of course, a satisfactory coloring can be attained using an electrolytic coloring bath having nickel sulfate concentrations outside the above range, but, in this case, it becomes difficult and economically unprofitable to practice the electrolytic coloring operation using an apparatus which is generally employed on an industrial scale. Also, as described above, the electrolytic coloring bath used in this invention can contain further boric acid, preferably at a concentration of 10 to 50 g/liter, for adjusting the electric conductivity of the bath whereby a more uniformly colored film can be obtained in a stable manner.

In the process of this invention, it is necessary that the pH of the electrolytic coloring bath is maintained at 2.0 to 5.5 since when the coloring treatment is conducted at a pH value outside the above range, the resulting color of the colored film becomes faint and the colored film tends to be peeled and spalled. That is, the coloring treatment cannot be conducted in a stable manner at a pH value outside the above range. Also, in a practical industrial operation, since a wide variety of bronze-like colors can be obtained uniformly and with better reproducibility by maintaining the pH of the electrolytic coloring bath in a range of 3.0 to 4.5, it is

possible to automate the electrolytic coloring operation. Therefore, it is preferable to maintain the pH of the electrolytic coloring bath in the range of from 3.0 to 4.5.

The procedure for the electrolytic coloring treatment is advantageously carried out using a current density in a range of 0.05 to 3.0 amperes/dm<sup>2</sup>, preferably 0.1 to 2.0 amperes/dm<sup>2</sup>.

The bath temperature can be room temperature with a satisfactory result, but the coloring operation can be conducted at a temperature in the range of from about 10 to about 40°C.

The time required for the electrolytic coloring treatment can be appropriately selected depending upon the color tone desired. Generally, as the period of time of electrolysis increases, the color of the film obtained becomes deeper. However, when a high current density such as about 2.0 amperes/dm<sup>2</sup> is employed in the electrolysis, a sufficiently deep color is obtained in a short period of time, e.g., 2 to 5 seconds and when a low current density such as 0.1 to 0.3 ampere/dm<sup>2</sup> is employed, a sufficiently deep color can be obtained at a comparatively longer period of time, e.g., 1 to 3 minutes.

On the other hand, from the practical standpoint, there is an inevitable tendency that the pH of the electrolytic coloring bath deviate from the preferred range of 3.0 to 4.5, even from the range of 2.0 to 5.5, upon continuing the electrolytic coloring operation on an industrial scale. This is due to the contamination of the electrolytic coloring bath with an anodic oxidation bath carried by the aluminum article or support members, great changes in the nickel ion concentration of the electrolytic coloring bath by the employment of materials which are not suitable as the anode in the electrolytic coloring bath, and the inadequate pH control of the electrolytic coloring bath. Therefore, in order to eliminate the above causes, it is required to strengthen the water rinsing after the anodic oxidation or to sufficiently rinse the aluminum article from the anodic oxidation treatment and the support members for the aluminum article by employing a water spray means and to use nickel having good solubility as the anode of the electrolytic coloring cell. Moreover, if the pH of the electrolytic coloring bath is inadequately controlled, it is necessary to immediately adjust the pH of the electrolytic coloring bath to the pH within the above range. That is, when the pH of the electrolytic coloring bath becomes too high, the pH can be easily reduced by adding a small amount of sulfuric acid to the electrolytic coloring bath and, on the other hand, when the pH of the electrolytic coloring bath becomes too low, the pH can be increased by dissolving a small amount of nickel hydroxide in the electrolytic coloring bath or passing the electrolytic coloring bath through an anion exchange resin. Thus, the pH of the electrolytic coloring bath can be maintained in the range of 2.0 to 5.5, preferably 3.0 to 4.5.

Procedures for increasing the pH of the electrolytic coloring bath will be described below in greater detail.

In the first procedure, the pH of the electrolytic coloring bath can be increased by dissolving nickel hydroxide as a neutralizing agent in the bath. Nickel hydroxide used in this procedure can be in the form of a powder or a paste. Generally, a small amount of nickel hydroxide will be sufficient. The neutralizing agent used in this procedure is not limited to nickel hydroxide, but on considering the influences of various metal

ions on the color of the colored film, the use of a nickel compound is preferred. Also, this procedure usually exhibits satisfactory results using nickel hydroxide at a concentration of from 10 to 1000 p.p.m. and, therefore, the pH control can be effected conveniently at low cost.

However, in practicing the neutralization, addition of alkalis which are generally used in the conventional neutralization procedure such as sodium hydroxide, potassium hydroxide, aqueous ammonia, etc. should be avoided in this invention since the contamination of the electrolytic coloring bath with alkali metal ions such as sodium ion, potassium ion or the like sometimes results in the spalling of the colored film on aluminum during the coloring treatment thereby adversely affecting the quality of the colored film. Further, when ammonium ions are present in the electrolytic coloring bath, a deep color cannot easily be obtained whereby the color is undesirably limited to specific colors.

In the second procedure, the pH of the electrolytic coloring bath which has decreased below 2.0 can be increased by treating the coloring bath with an anion exchange resin. In this case, the use of a weak basic anion exchange resin is most preferable since free sulfuric acid is mainly removed by the anion exchange resin and thus the pH of the electrolytic coloring bath can be readily adjusted to a value in the desired pH range.

The invention will be further explained in greater detail by referring to the following Examples but these Examples are not to be construed as limiting the scope of this invention. Unless otherwise indicated, all parts, percents, ratios and the like are by weight.

#### EXAMPLE 1

An aluminum plate (99.2% Al) was immersed in an aqueous 10% sodium hydroxide solution at 60°C for 2 minutes, and then subjected to a neutralization treatment with a 20% aqueous nitric acid solution at room temperature. After rinsing the aluminum plate with water, it was subjected to an anodic oxidation treatment in a 15% aqueous sulfuric acid solution for 15 minutes at a current density of 2 amperes/dm<sup>2</sup> and at a bath temperature of 20±1°C. The anodized aluminum plate thus obtained was then subjected to electrolytic coloring treatment as a cathode with a direct current in an electrolytic coloring bath containing 50 g/liter of nickel sulfate and 30 g/liter of boric acid for 1 minute at a current density of 0.3 ampere/dm<sup>2</sup> and at a bath temperature of 20±1°C using a nickel plate as an anode. In this case, the pH of the above electrolytic coloring bath was reduced to 1.5 using sulfuric acid and then the pH of the electrolytic coloring bath was gradually increased to 5.7 by dissolving nickel hydroxide therein, whereby the electrolytic coloring treatment was conducted at various pH values of the bath.

The color lightness of the resulting aluminum plates which have been colored at various pH values of the electrolytic coloring bath was then evaluated using an integrating automatic colorimetric color-difference meter type AU-SCH-2 (made by Toyo Rika Kogyo K.K.), and the results obtained are shown in Table 1. The values in Table 1 below are shown in terms of the lightness in the Munsell color system (V<sub>y</sub>). When the color of the bronze-like colored film on the aluminum is shown in terms of the value in the Munsell color system, a value above 5.0 indicates the color of aluminum itself and a value in the range of from 4.0 to 5.0

indicates a very faint color tone. At a value below 4.0, the color of the film becomes deeper as the value lowers, and, at about 1.5, the color is very deep.

What is claimed is:

1. In a process for electrolytically coloring an anodically oxidized coating on an aluminum or aluminum

Table 1

| pH                             | 1.5  | 2.0  | 2.3  | 2.6  | 3.0  | 3.5  | 4.1  | 4.5  | 4.9  | 5.4  | 5.7 |
|--------------------------------|------|------|------|------|------|------|------|------|------|------|-----|
| Lightness<br>(V <sub>Y</sub> ) | 5.21 | 3.88 | 2.70 | 2.20 | 2.12 | 2.03 | 1.91 | 1.87 | 2.03 | 4.85 | —*  |

\*The colored film was spalled at the pH of 5.7.

As is clear from the results shown in Table 1, it is necessary that the pH of the electrolytic coloring bath be in the range of 2.0 to 5.5.

#### EXAMPLE 2

An aluminum plate (99.2% Al) was subjected to the same pre-treatment and anodic oxidation treatment as in Example 1, and then subjected to an electrolytic coloring treatment with a direct current in an electrolytic coloring bath containing 35 g/liter of nickel sulfate and 35 g/liter of boric acid for 2 minutes at a current density of 0.3 ampere/dm<sup>2</sup> and at a bath temperature of 20 ± 1°C using the anodized aluminum plate as a cathode and a nickel plate as an anode. In this case, the electrolytic coloring was effected using the electrolytic coloring bath having a pH of 1.5 adjusted with sulfuric acid, and then the electrolytic coloring bath was passed through a weak basic anion exchange resin, Duolite-A6 (Registered Trade Mark: Diamond Shamrock Corp.) at various space velocities to increase the pH of the bath whereby the electrolytic coloring treatment was performed at various pH values of the electrolytic coloring bath. The color lightness of the resulting colored aluminum plates was evaluated as described in Example 1, and the results obtained are shown in Table 2 below.

Table 2

| pH                             | 1.5  | 2.0  | 2.5  | 3.0  | 3.5  | 4.0  | 4.5  | 5.0  | 5.5  | 5.7 |
|--------------------------------|------|------|------|------|------|------|------|------|------|-----|
| Lightness<br>(V <sub>Y</sub> ) | 5.50 | 3.29 | 1.61 | 1.57 | 1.43 | 1.29 | 1.52 | 2.10 | 4.91 | —*  |

\*The colored film was spalled at the pH of 5.7.

As is clear from the results shown in Table 2, the suitable pH value ranges from 2.0 to 5.5, and more preferably from 3.0 to 4.5. In addition, it was confirmed that the concentrations of the nickel sulfate and boric acid in the electrolytic coloring bath are not substantially influenced by passing the coloring bath through the ion exchange resin.

While the invention has been described in detail and with reference to specific embodiments thereof, it will be apparent to one skilled in the art that various changes and modifications can be made therein without departing from the spirit and scope thereof.

alloy article comprising subjecting said article to anodic oxidation in an aqueous anodic oxidation bath consisting essentially of sulfuric acid or an aromatic sulfonic acid to form an oxidized film of a thickness of

15 at least 6 microns and electrolyzing said anodic oxidized article as a cathode immersed in an aqueous electrolytic coloring bath containing a water-soluble nickel salt selected from the group consisting of nickel sulfate, nickel chloride and nickel acetate using a direct current, the improvement of obtaining uniformly colored coating on the aluminum article by maintaining the pH of said electrolytic coloring bath in a range of from 2.0 to 5.5 during said electrolytic coloring treatment.

20 2. The process according to claim 1, wherein said nickel salt is nickel sulfate.

3. The process according to claim 1, wherein said electrolytic coloring bath further contains boric acid.

4. The process according to claim 1, wherein the pH 30 of the electrolytic coloring bath is maintained at 3.0 to 4.5 during said electrolytic coloring treatment.

5. The process according to claim 1, wherein the pH of the electrolytic coloring bath is maintained at 2.0 to 5.5 by adding a small amount of sulfuric acid to the bath.

45 6. The process according to claim 1, wherein the pH of the electrolytic coloring bath is maintained at 2.0 to 5.5 by adding a small amount of nickel hydroxide to the bath.

7. The process according to claim 1, wherein the pH of the electrolytic coloring bath is maintained at 2.0 to 5.5 by passing the electrolytic coloring bath through an anion exchange resin.

50 8. The process according to claim 7, wherein said anion exchange resin is a weak basic anion exchange resin.

\* \* \* \* \*